

## UNITED STATES PATENT OFFICE

ERICH WIEGAND, OF BERLIN-WAIDMANNSLUST, GERMANY, ASSIGNOR TO GENERAL ELECTRIC COMPANY, A CORPORATION OF NEW YORK

## MANUFACTURING OXIDE CATHODES

No Drawing. Application filed June 30, 1931, Serial No. 548,036, and in Germany July 16, 1930.

One known method of manufacturing oxide cathodes consists in precipitating alkaline-earth metal from the vapor phase onto an unheated carrier filament and oxidizing the said metal by subsequently heating the carrier filament in oxygen, for the purpose of obtaining alkaline earth oxide. While this process may produce cathodes of relatively long life and high electron emissivity, it has been found that notwithstanding the extreme care exercised in their manufacture, such cathodes are not accurately reproducible on a quantity production basis, in so far as their electron emission is concerned. All attempts made to the present day to obviate this disadvantage have not been entirely successful and no satisfactory explanation has been offered for this failure. However, in accordance with my invention, cathodes of considerably greater uniformity are obtained when the filament is activated by following another procedure. The new process consists in coating the cathode carrier with an oxygen compound and heating the carrier to such a temperature when the alkaline-earth metal is in the form of vapor that no appreciable quantity of alkaline-earth metal (in solid or liquid form) is deposited on the said carrier, but the conversion takes place exclusively between the oxygen compound on the carrier and vaporized alkaline-earth metal. The purpose of the invention is best served by using those oxygen compounds which are still sufficiently stable at a temperature exceeding about 900° C. and in a vacuum. Good results may be obtained with tantalum oxide and lower tungsten oxides. The temperature to which the cathode must be heated when the metal is in the vapor state depends upon the nature of the alkaline-earth metal used. A temperature of the order of 900° C. is generally sufficient when using barium metal, but must be somewhat higher in the case of calcium and strontium owing to their relatively low vapor pressures.

Since according to the new process, neither liquid nor solid, as distinguished from gaseous alkaline-earth metal can reach the filament, there are no disturbing electron emission effects on cathodes manufactured according to the improved process. There are also no changes of electron emissivity throughout the length of the coating caused by alkaline-earth metal condensing on the surface of the filament and flowing to the cold ends thereof. This may be the reason for the greater uniformity of the improved cathodes in respect to their electron emission properties. Particularly desirable results are obtained by heating the cathode to such a temperature, when the alkaline-earth metal vapor is being evolved, that the oxygen compound is partially evaporated or decomposed. This method yields cathodes having extremely high electron emissivity.

What I claim as new and desire to secure by Letters Patent of the United States, is:—

1. A process of manufacturing cathodes for electric discharge devices, said process including the steps of applying an oxygenous compound to a cathode foundation member and heating the oxidized member in the vapor of an electronically active material to a temperature so high that the said material is precluded from forming on the foundation member in a solid or liquid state.

2. A process of manufacturing cathodes for electric discharge devices, said process including the steps of coating a foundation metal of the cathode with an oxygen compound and heating the coated metal in the vapor of an alkaline earth metal to a temperature exceeding 900° C. whereby the said metal is precluded from forming on the foundation member in solid or liquid state.

3. A process of manufacturing cathodes for electric discharge devices, said process including the steps of applying a dissociable oxygenous compound to the surface of a cathode foundation member and heating said

member in the vapor of an alkaline earth metal to a temperature so high that the said compound becomes partially decomposed and the alkaline earth material combines with the oxygen on the oxidized surface.

5 4. A process of manufacturing cathodes for electric discharge devices, said process including the steps of coating a foundation metal with tantalum oxide and heating the coated member in the presence of an alkaline earth vapor to a temperature of the order of 900° C.

10 In witness whereof, I have hereunto set my hand.

15

ERICH WIEGAND.

20

25

30

35

40

45

50

55

60

65